

# UNITED STATES PATENT OFFICE.

GEORGE G. TAYLOR, OF HOLYOKE, MASSACHUSETTS, ASSIGNOR TO AMERICAN WRITING PAPER COMPANY, OF HOLYOKE, MASSACHUSETTS, A CORPORATION OF NEW JERSEY.

## PROCESS OF BLEACHING VEGETABLE FIBERS.

1,381,440.

Specification of Letters Patent. Patented June 14, 1921.

No Drawing.

Application filed December 18, 1920. Serial No. 431,794.

To all whom it may concern:

Be it known that I, GEORGE G. TAYLOR, a citizen of the United States, residing at Holyoke, in the county of Hampden and State of Massachusetts, have invented certain new and useful Improvements in Processes of Bleaching Vegetable Fibers, of which the following is a specification.

This invention relates to the art of bleaching vegetable fibers, and comprises a novel process whereby such fibers may be quickly bleached without injurious effect due to the bleaching agent.

It has long been recognized that hypochlorous acid, owing to the comparative readiness with which it parts with oxygen, is a much more energetic and rapid bleaching agent than any of its salts. Accordingly it is customary, in employing hypochlorites as bleaching agents, to introduce into the bath at some stage of the operation an acid or acid salt in order to liberate free hypochlorous acid.

In the textile industry this is accomplished by passing the cloth saturated with the hypochlorite bleaching solutions into a bath of dilute acid. The paper maker, who is obliged to bleach his material in the form of pulp, adds acid or an acid reacting salt to the washing engine, or to such other apparatus as may be employed for bleaching, before the bleach liquor is exhausted. The acids most commonly used in both industries are sulfuric and acetic acids, while sulfate of aluminum is the salt usually employed.

The disadvantage of the addition of any of the above materials as now commonly employed consists first in the fact that when hypochlorous acid gives up its oxygen in the course of the bleaching operation, hydrochloric acid is formed; and hydrochloric acid even in very dilute solution has an injurious action upon cellulose fibers; and second, in the fact that the addition of an excess of any of these materials decomposes the hypochlorite with evolution of chlorin, which is not a primary bleaching agent.

According to the present invention these difficulties are overcome by adding to the bleaching bath, comprising any of the salts of hypochlorous acid, boric acid in less than the equimolecular proportion to the hypochlorite present. The boric acid liberates hypochlorous acid from a portion of the

hypochlorite, a corresponding quantity of 55 borate being of course formed; the latter salt is however at once decomposed by the hydrochloric acid resulting from the decomposition of the hypochlorous acid, whereby boric acid is again set free, and the cycle 60 repeated until the whole of the hypochlorite has been utilized in the form of free hypochlorous acid.

Assuming sodium hypochlorite to be the bleaching agent employed, and a small proportion of boric acid to be added during the bleaching operation, the cycle of ensuing reactions may be represented as follows:



The regenerated boric acid will go through the cycle of reactions as long as any hypochlorite remains.

In the case of calcium hypochlorite the reactions will be similar, viz:



In either case it will be noted that the boric acid is regenerated, and therefore that a small amount of it will be sufficient to liberate all the hypochlorous acid contained in a large amount of bleaching powder or of 95 sodium hypochlorite. In actual practice I prefer to use about one pound of boric acid for each 100 pounds of paper stock, but my invention is of course not limited to this approximate proportion.

I claim:

Process of bleaching vegetable fibers, comprising subjecting the fiber to a hypochlorite in presence of free boric acid, the latter in less than the equimolecular proportion to 105 the hypochlorite.

In testimony whereof I affix my signature.  
GEORGE G. TAYLOR.